

## UNITED STATES PATENT OFFICE

SAMUEL S. SADTLER, OF CHESTNUT HILL, SPRINGFIELD TOWNSHIP, MONTGOMERY COUNTY, PENNSYLVANIA, ASSIGNOR TO AMIESITE ASPHALT COMPANY OF AMERICA, OF PHILADELPHIA, PENNSYLVANIA, A CORPORATION OF NEW JERSEY

## COATING DAMP OR WET STONE

No Drawing.

Application filed August 18, 1927. Serial No. 213,973.

This invention relates to improvements in the art of road making, and the principal object of the invention is to provide novel and improved means for coating damp stone, constituting the aggregate of which the road composition is made, with asphalt or other bitumen.

It is frequently desirable to make roadways of the general type set forth in U. S. Patent No. 1,611,444 without special drying of the stone or the aggregate in preparation for coating the stone with bitumen. Difficulty, however, has been experienced in the absence of the drying operation of obtaining a satisfactory bond between the bitumen and the surfaces of the stone. It has been particularly difficult to obtain satisfactory results under the stated circumstances in connection with roadways or surfaces in which

the voids between the bitumen-coated stones are not filled and in which the stones are cemented together solely or principally by their asphaltic or bitumen coatings.

In co-pending applications Nos. 89,762 and 178,814, I have made use of sulphonated oils and compounds of oleic acid more or less saponified, to effect a coating of damp or wet stone. There are certain reasons why, for sake of economy, and a desire to add nothing organic to the asphalt, it is desirable to use inorganic substances to effect this coating of damp or wet aggregate.

I have discovered, therefore, that by the use of an extremely colloidal clay, such as bentonite, the coating may be effected without the use of soaps, sulphonated oils or acid oleates.

In practice, I apply this powdered colloidal clay (or bentonite) to damp or wet stone in the mixer or pug mill, and turn it until the bentonite is thoroughly dispersed on the surfaces of the stone. From practical trials, I have found that it takes about 0.15% of a good grade of bentonite, based upon the weight of the stone. This amount, however, is more or less dependent upon the amount of water in the stone, the amount added will vary in practice from 0.2 per cent to 0.4 per cent, depending upon the character of the stone, and the character of service

to which the road will be subjected. The test referred to was with stone containing 2% of water by actual test. This makes the figure of 0.15% on the weight of the stone 7.5% on the water content of the stone.

After finding that 5% on the weight of the water was insufficient, I made a series of surface tension tests, and found that 5% was below the surface tension of the water used, and 7.5% was slightly above it. It would seem, therefore, that a figure of 7.5% was close to a practical amount to use; the amount added will vary in practice from 5% to 8% of the moisture in the stone determined by analysis, and will also be influenced by the character of the service to which the road will be subjected. I, however, claim the right to vary the quantity in accordance with what I find necessary to use to accomplish the desired results.

After the addition of the bentonite, I proceed in the usual way for making stone-asphalt paving compositions by the use of a liquefier, such as kerosene or naptha, or suitable mixtures of these materials, and prefer to use hydrated lime immediately after the addition of the melted asphalt.

Because of the chilling effect of the water, it is necessary to have the asphalt well heated. It should be close to 300° F., but not above this figure, as the asphalt, itself, would be endangered by the high heating.

I prefer to use from 5 to 10 pounds of hydrated lime per ton mix.

If it is desirable to add some sandy fines to the mix, they may be added after the asphalt is thoroughly mixed.

The amount of asphalt used is approximately the same as in ordinary dry coating, and varies with the size of the stone from about 80# for coarser stone to 120 or 130 pounds per ton of finished product for finer grades. There need be no change in the penetration of the asphalt as compared with the dry coating. I prefer to use asphalt of approximately 100 penetration. For warm climates, it is desirable to lessen the penetration. It may be as much as 20° as compared with the temperate climates.

## Claims:

1. The method of preparing a paving material from damp stone, which comprises agitating said stone in a mixer and dispersing upon said agitated stone a thin coating of highly colloidal clay, thereafter adding a volatile hydrocarbon to the mass of agitated coated stone and distributing said hydrocarbon over said coated stone, thereafter adding hot asphalt to the mass and continuing the agitation until the asphalt has been distributed over said coated stone. 70
2. The method of preparing paving material from damp stone, which comprises agitating said stone in a mixer, dispersing highly colloidal clay upon said agitated stone as a thin coating, said clay constituting a variable amount, and may vary from about 0.2 per cent to 0.4 per cent of the weight of the finished batch of paving material, adding a volatile hydrocarbon to the agitated coated stone, and thereafter adding hot asphalt to the mass, and continuing the agitation until the asphalt has been distributed over said coated stone. 75
3. The method of preparing paving material from damp stone, which comprises agitating said stone in a mixer, dispersing highly colloidal clay upon said agitated stone as a thin coating, said clay constituting a variable amount, and may vary from 5 percent to 8 percent of the weight of the water contained in the stone, adding a volatile hydrocarbon to the agitated coated stone, and thereafter adding hot asphalt to the mass, and continuing the agitation until the asphalt has been distributed over said coated stone. 80
4. The method of preparing a paving material from damp stone, which comprises agitating said stone in a mixer and dispersing upon said agitated stone a thin layer of bentonite, thereafter adding a volatile hydrocarbon to the mass of agitated coated stone and distributing said hydrocarbon over said coated stone, thereafter adding hot asphalt to the mass and continuing the agitation until the asphalt has been distributed over said coated stone. 85
5. The method of preparing paving material from damp stone, which comprises agitating said stone in a mixer, dispersing bentonite upon said agitated stone as a thin coating, said bentonite constituting a variable amount, and may vary from about 0.2 percent to 0.4 percent of the weight of the finished batch of paving material, adding kerosene to the agitated coated stone, and thereafter adding hot asphalt to the mass, and continuing the agitation until the asphalt has been distributed over said coated stone. 90
6. The method of preparing paving material from damp stone, which comprises agitating said stone in a mixer, dispersing bentonite upon said agitated stone as a thin coating, said bentonite constituting a variable amount, and may vary from 5 percent to eight per cent of the weight of the water contained in the stone, adding kerosene to the agitated coated stone, and thereafter adding hot asphalt to the mass, and continuing the agitation until the asphalt has been distributed over said coated stone. 95

In testimony whereof I affix my signature. 100  
SAMUEL S. SADTLER.